

Aug. 28, 1928.

1,682,076

J. O. GOGRY

PROCESS OF PROTECTING ELECTRIC AND OTHER CABLES

Filed Nov. 14, 1925

Fig. 1



Fig. 2



Fig. 3



INVENTOR:

*Jean Octave Gogry*  
BY  
*John J. Murphy, Jr.*  
ATTORNEY

## UNITED STATES PATENT OFFICE.

JEAN OCTAVE GOGRY, OF VINCENNES, FRANCE.

## PROCESS OF PROTECTING ELECTRIC AND OTHER CABLES.

Application filed November 14, 1925, Serial No. 69,062, and in France November 27, 1924.

Electric conductors at present in use are insulated either with india-rubber (for industrial tensions), or with paper or cotton (for the low tensions employed in telephony, 5 telegraphy, machine element constructions etc.).

Such materials, however, offer the drawback of being affected by numerous agents which reduce their insulating action to such 10 a degree that plant safety does not permit the conductors to be kept in service for long without serious risks.

Chiefly dangerous among the said destructive agents can be mentioned:

15 1. Moisture at any temperature.

2. Dry heat above 100° C.

3. Chemicals, either per se or through their emanations, (acids, strong bases, alkalies etc.).

20 4. Certain products commonly met with in industry (spirits, oil etc.).

The object of my invention is to provide a process for insulating electric or other cables, whatever their form and section, and

25 whatever their contexture, rendering them capable of resisting and withstanding in an efficient and long durable manner the action of the above mentioned destructive agents.

My invention also covers the various baths 30 and the apparatus employed in carrying out the said process.

In the following specification I will begin by describing, as an example, a method of coating electric cables adapted to withstand 35 the above recited agents, except, however, concentrated acids. I will afterwards disclose means for rendering said cables resistant to such acids, and, lastly, I will describe, merely as an example, or as an indication, 40 an embodiment of an apparatus for performing my process.

Electric conductors are generally covered with unbleached cotton plaiting, fairly loose but very smooth and even.

45 I pass such conductors through a hot bath very heavily charged with drying oil. Such a bath may be prepared, for instance, by heating to about 110° C., in a vat having a capacity substantially greater than the volume 50 of its contents, the following substances:

Per cent.

Drying oil..... 45  
Gum resin..... 10

55 Pulverulent inert mineral matter..... 45

Stirring the whole thoroughly so as to obtain a homogeneous mixture.

On removal from the bath, I draw the conductors through a calibrated draw-plate, the purpose of which is to leave only a mere film 60 of coating on their surface.

This first bath is intended to fill and close the meshes of the braided cotton or other fabric insulation with an inert material, at the same time shrinking the cotton through 65 oxidation of the oil, thereby proofing the backing and facilitating application of the coatings to be superadded thereon.

I make loose bundles of the so-treated conductors and leave them exposed to free air for 70 drying, which takes practically from 4 to 8 days.

Once they are thoroughly dry, I pass them through a second hot bath, very heavily charged with gum, which bath may be prepared by heating to about 110° C., in a vat similar to the first one, the following substances:

|                                       | Per cent. |
|---------------------------------------|-----------|
| Drying oil.....                       | 5         |
| Gum resin.....                        | 30        |
| Paraffin.....                         | 30        |
| Pulverulent inert mineral matter..... | 35        |

Stirring the whole so as to obtain a homogeneous mixture.

On removing them from this bath, I draw the conductors through a calibrated draw-plate having holes about 5 to 10% larger in diameter than the first one.

Said conductors, so treated, dry very rapidly, and I then subject them to "glazing".

This operation, which constitutes one of the essential characteristics of my invention, consists in drawing the conductors through a calibrated draw-plate, preferably made of steel, suitably heated (practically to over 100° C.) and having holes of smaller diameter than those of the draw-plate utilized after the second bath.

The purpose of such operation is:

1. To force into and compress in the very smallest interstices the constituent materials;
2. To melt the second coating, very heavily charged with gum, and to combine it with the first one, very heavily charged with already very much oxidized oil, thereby forming in situ and within the very body of the backing and conductor-surrounding fabric, a continuous sheath of coating, (very similar to

100

105

110

oil varnishes), which will proof the conductor in a positive manner:

3. To impart to the whole a flexibility permitting any bendings, which are unavoidable in utilization of electric conductors, without any risk of cracking or breaking:
- By forming the flexible final coating,
  - By eliminating any superfluous quantities of the second coating product, always 10 very brittle.

In order to obtain conductors proofed to withstand cold moisture and concentrated acids, I proceed in the same manner as above, (heating to about 110° C. and stirring) but 15 the second bath is composed of the following substances:

|                                  | Per cent. |
|----------------------------------|-----------|
| Drying oil                       | 5         |
| Gum resin                        | 20        |
| Asphalt                          | 10        |
| Paraffin                         | 30        |
| Pulverulent inert mineral matter | 30        |

Furthermore, after glazing, I pass the conductors through a last bath, prepared like 25 the preceding ones, but composed of the following substances:

|                                  | Per cent. |
|----------------------------------|-----------|
| Asphalt                          | 50        |
| Paraffin                         | 25        |
| Vaseline                         | 5         |
| Pulverulent inert mineral matter | 20        |

On removing them from this last bath, I draw the conductors through a calibrated 35 draw-plate, the holes of which are just of sufficient diameter to leave on their surface a coating 0.1-0.2 mm. thick.

The conductors will then dry very rapidly, and be ready for service.

40 In order to make the method of performing my said invention more clearly understood, I have illustrated, as an example, an apparatus adapted for this purpose in the accompanying drawing, wherein:

45 Figure 1 is a diagram affording a general view of a conductor-coating device;

Figure 2 illustrates the supporting and heating arrangement of the glazing draw-plate;

50 Figure 3 shows a draw-plate on an enlarged scale.

I prepare the baths in vats, preferably gas heated, and which may be provided with stirrers or agitators.

55 Coating is performed in troughs, such as the one shown at A on Figure 1, heated by any suitable gas, electric or other device B.

The cable to be coated is initially wound around a reel C, supported by a frame D on 60 which said reel is adapted to revolve, and passes therefrom over a guide roller E, then dips into the bath contained in trough A, wherein it is maintained by a plunger F fitted with a roller, and comes out at the opposite end of the trough. The cable passes next

through draw-plate H, combined with a guiding device E<sup>2</sup>, and is wound up on a suitable device, say a reel or a spool.

For glazing, draw-plate H is mounted on a holder or stand D' (Figure 2). I heat it 70 up to suitable temperature by means of a device B', preferably a gas burner.

The draw-plates are made of steel, and, preferably, rectangular in shape, as shown by Figure 3. The draw-hole should have its 75 lowest part at a constant distance from the base so as to ensure perfect centering, and the entrance aperture of said hole should be countersunk, as indicated at I.

The above described apparatus is given, of course, simply as an example in order to render the invention more clearly understandable, and it is, therefore, in no way limitative and I reserve the right to introduce any 85 constructional modifications without being deemed to depart from the scope of my said invention.

I claim as my invention:

1. A process of treating insulated electric and other cables, comprising the steps of 90 passing the cable through a hot drying-oil bath and then subjecting it to a drawing action, so as to leave merely a thin film of coating on the surface of the insulation; drying the coated cable; passing it through a hot gum bath and then subjecting it to a second drawing action; and then subjecting the cable, after having undergone the second drawing action, to a drawing action in the presence of heat to cause the constituent materials of the two baths to combine and to force them into the interstices of the insulation.

2. A process of treating insulated electric and other cables, comprising the steps of 105 passing the cable through a hot drying-oil bath and then subjecting it to a drawing action, so as to leave merely a thin film of coating on the surface of the insulation; drying the coated cable; passing it through a hot gum bath and then subjecting it to a second drawing action; and then glazing the cable.

3. A process of treating insulated electric and other cables, comprising the steps of passing the cable through a hot drying-oil bath 115 and then subjecting it to a drawing action, so as to leave merely a thin film of coating on the surface of the insulation; drying the coated cable; passing it through a hot gum bath and then subjecting it to a second drawing action; glazing the cable; and then subjecting the glazed cable to acid proofing.

4. In a process of treating insulated electric and other cables, the steps of passing the cable first through a hot drying-oil bath, and subsequently through a hot gum bath containing drying oil, gum resin, paraffin and pulverulent inert mineral matter.

5. In a process of treating insulated electric and other cables, the step of passing the 120

cable first through a hot bath containing drying oil, gum resin and pulverulent inert mineral matter, and then through a hot gum bath containing drying oil, gum resin, paraffin and 5 pulverulent inert mineral matter.

6. A process, according to claim 5, in which the cable, after having been passed through the second bath, is dried and then subjected to drawing action in the presence of heat to 10 cause the constituent materials of the two baths to combine.

7. In a process of treating insulated electric and other cables, the steps of passing the cable first through a hot drying-oil bath and then through a hot gum bath, glazing the 15 coated cable after it has been passed through the gum bath, and then subjecting it to a bath for proofing it against concentrated acids.

In testimony whereof I affix my signature.

JEAN OCTAVE GOGRY.